

June 8, 1948.

H. W. MORREALL, JR

2,442,930

PROCESS FOR DEVELOPING MULTILAYER FILM CONTAINING COLOR FORMERS

Filed Sept. 29, 1944



INVENTOR  
Herbert W. Morreall Jr.  
BY *Henry M. Langley*  
Lewis D. Konigford  
ATTORNEY

## UNITED STATES PATENT OFFICE

2,442,930

## PROCESS FOR DEVELOPING MULTILAYER FILM CONTAINING COLOR FORMERS

Herbert W. Morreall, Jr., Binghamton, N. Y., assignor to General Aniline & Film Corporation, New York, N. Y., a corporation of Delaware

Application September 29, 1944, Serial No. 556,324

3 Claims. (Cl. 95—2)

1

The present invention relates to improvements in multilayer color films and to the process of development thereof, and relates in particular to multilayer color film adapted for reversal development.

Multilayer color films containing color formers in the respective layers and adapted to be developed by the reversal process, generally consist of a suitable backing or support upon which is a number of layers, the first, for example, being a gelatino silver halide emulsion sensitized to red light and containing a nondiffusing color coupling component capable of being developed in a suitable color developer to a cyan colored image; the second being a gelatino silver halide emulsion sensitized to green light and containing a nondiffusing color coupling component capable of being developed in a suitable color developer to a magenta image; and the third being a gelatino silver halide emulsion sensitized to blue light and containing a color coupling component capable of being developed with a suitable color developer to a yellow image. Suitable nondiffusing color coupling components are disclosed in U. S. Patents 2,179,238, 2,186,733, 2,224,329 and 2,178,612. Generally, also, between the second and third layers is interposed a suitable yellow filter layer the color of which is destroyed in the silver bleaching bath. Other kinds of color films containing color formers in the respective layers, are also known.

In the reversal process of producing colored photographs, which is referred to herein to illustrate the invention, the multilayer color film having the color formers contained within the respective layers, after initial exposure to light from the subject to be photographed, is first developed with a noncolor forming developer to produce a silver negative, then the film is removed from the developer and re-exposed to white light, and thereafter the film is developed to develop the color formers. Finally the reduced silver is removed from the film by a suitable silver solvent. In this process difficulty heretofore has been encountered in obtaining adequate negative development of the lowermost layers in the film. For example, in a typical multicolor tri-pack film in which the cyan layer is the lowermost layer, the development of color film as above described tends to result in a decrease in effective sensitivity or photographic speed of the film, and also results in excessive green highlights in the film on developing of the colored image. Attempts to overcome this difficulty by extending the time of the first develop-

2

ment have not produced satisfactory results because this causes overdevelopment and reduction in contrast in the image in the uppermost layers.

It is an object of the present invention to provide an improved multilayer color film containing the color formers within the several layers having an increased photographic speed.

Another object of the invention is to provide an improved multilayer reversal color film containing the color formers within the several layers which results in an increase of speed of the color film and reduction of the green highlights in the reversal development.

Another object is to reduce the time required for developing multilayer color film containing the color formers within several layers.

Another object is the provision of a developing process for multilayer color film whereby the development may be carried out at temperatures below normal room temperature, or at normal room temperature in a shorter time.

In accordance with the present invention, I have found that the development of an exposed multilayer color film in the presence of a compound of the general formula:



30 wherein X represents hydrogen, a saturated or unsaturated aliphatic hydrocarbon radical, or the cyanide radical, overcomes the difficulties heretofore experienced and results in an increase in speed of the multicolor film. In particular in the 35 reversal development process the lowermost layer in a tri-pack film, which is the cyan layer, is benefited by reduction of the green highlights. The green highlights are believed to be caused by incomplete development of the image in the 40 lower layer in the first or negative development so that undeveloped silver remains and reacts in the color forming development to produce color in those parts of the layer where there should be no color. When the film is viewed through white 45 light the cyan layer allows green to pass through and thus produces a green highlight. Similar beneficial results are obtained in developing multilayer color negative films in the presence of said compounds according to the present invention, particularly when the urea compound is incorporated in the emulsion.

In particular I prefer to employ the N-hydrocarbon substituted ureas corresponding to the above formula in which X represents a saturated or unsaturated aliphatic hydrocarbon group, as

for example the allyl or the methyl group, such compounds being represented by the following formula:



where Z represents an aliphatic hydrocarbon radical, as for example, methyl- or allyl-. In general, urea itself is more active than the substituted compounds in the above formula, and larger quantities of the substituted compounds are required to produce the beneficial effects of urea. For simplicity of expression in the following description of the invention the term urea compound will be employed to generically designate the substances included in the above formula.

The urea compound referred to herein may be present in the various gelatin emulsion layers of the film, or may be added to the developing solution employed in the first or negative development with satisfactory results. It is believed that the urea compound acts as a swelling agent upon the gelatin emulsion to allow faster and better penetration of the developer, and this is accomplished without undue permanent softening or other undesirable results. When added to the developer solution it accelerates the development of all layers and particularly that of the lowermost layer and has little if any deleterious effect on the stability of the solution. Also the maximum color density, the gradation or contrast of the developer film and the effect upon the grain size of the final dye image is not substantially adversely affected. Furthermore it has no permanent softening effect on the emulsion, for it is washed out by the subsequent treatment in the development of the film so that the film resumes substantially its original hardness.

In employing a urea compound in the gelatin emulsion a concentration of about one to ten grams per kilogram of emulsion may be employed. Optimum effects with urea generally are obtained with a concentration of about 4 to 6 grams per kilogram of wet emulsion, or about 4 to 6 percent of the dry emulsion. Such emulsions it will be understood, contain suitable color sensitizers and color formers, the urea being added to the emulsions preferably after the washing operation and just prior to the coating of the emulsion layers on the support.

The quantity or concentration of urea compound in the developer solution required for obtaining results depends, among other things, upon the initial hardness of the gelatin in the emulsion layers and upon the temperature at which the development takes place. For the development at room temperature, I have found that a concentration of about 65-75 grams urea per liter of developer solution is sufficient although in developing unusually hard gelatin layers I may use 100, 125 or 150 grams urea per liter, and for softer emulsions I may use as low a concentration as 25 grams of urea per liter. Corresponding quantities of the other urea compounds above referred to may be employed. Too high a concentration of urea is to be avoided for it has a tendency to produce softening and reticulation of the emulsion. Urea has very little effect on the pH value.

The advantages pointed out above in particular are secured where the first development of the multilayer color film is carried out with amidol, which is a preferred developer. Alkali in

a developer is known to have a softening action on the gelatin, but alkali rapidly deteriorates amidol developer. Thus in the use of amidol as a developer, it is necessary to avoid a high pH value in the solution, and this may be accomplished by the addition of the urea compounds to the developer solution which accelerates the effect of the developer without unduly increasing the pH value of the solution. However, it will be understood that the beneficial effects of the present invention are not limited to the use of amidol as the developer, as other developers known in the art may be employed.

If desired the beneficial effect of urea may be availed of by carrying out the development at lower than room temperature or by carrying out the development at room temperatures for shorter periods of time.

The invention will be explained in greater detail in connection with the following examples and accompanying drawing which are cited to illustrate the invention, and wherein:

Figure 1 illustrates a preferred embodiment of color film incorporating the invention and

Figure 2 illustrates by representative graphs the speed increase in the layers of a multilayer color film.

Referring to Figure 1 wherein is shown one embodiment of color film, the numeral 1 represents a suitable support, such as a cellulose ester film which carries a suitable emulsion layer 2 sensitized to red light by a suitable sensitizer and containing a suitable complementary color former such as 3,5-di(phenylamino) phenol which is capable of being developed in a suitable color developer such as p-diethylamino aniline to produce a cyan image. The emulsion layer 3 superposed on layer 2 is sensitized to green light by a suitable sensitizer and contains a suitable complementary color former, such as p-(oxynaphthoylamino)-1-phenyl-3-methyl-5-pyrazolone capable of being developed to a magenta image. Interposed between layers 3 and 5 may be a yellow filter layer 4, such as a gelatin layer colored with Benzo Fast Yellow RL, C. I. 349A or any other suitable yellow coloring matter. If desired, this filter layer may be omitted. Layer 5 is sensitive to blue light and contains a suitable complementary color former, such as terephthaloyl-bi-acetic acid anilide capable of being developed to a yellow image. The emulsions may be prepared, for example, as described in U. S. Patent 2,179,238, and about 4 to 6 grams urea per kilogram of emulsion are added after the washing operation just prior to applying the emulsion layers to the support.

#### Example 1.—Tri-pack color film

An exposed tri-pack color film is developed in a developer solution composed, for example, of 5 grams amidol, 50 grams sodium sulfite crystals and 2 grams potassium bromide in a liter of water to which is added 75 grams of urea, the film being developed in this solution for about 20 minutes. The development is then arrested and the film exposed to white light, and thereafter the film is developed in a color forming developer solution containing, for example, diethyl-p-phenylenediamine, which produces positive silver images simultaneously with the formation of colored dye images. All the silver then is bleached to metallic silver, and the metallic silver from each layer is removed with Farmer's solution leaving pure dye images in natural color. The positive produced in this way shows

an absence of undue green highlights and results in a clearer image as compared to the film developed without urea.

Other known developers may be used with a suitable quantity of a urea compound, as for example, a metolhydroquinone developer containing metal 4 grams, sodium sulfite 40 grams, hydroquinone 4 grams, sodium carbonate 40 grams, potassium bromide 2 grams and potassium thiosulfate 2 grams in a liter of solution; or a glycine 10 developer containing glycine 7.5 grams, sodium carbonate 50 grams, potassium bromide 2 grams and potassium thiosulfate 2 grams per liter.

*Example II.—Multilayer color negative film*

The exposed multilayer film with color formers in the several layers is developed for approximately 15 minutes at a temperature of about 68° F. in a developing bath containing per liter the following concentrations: 2 grams sodium sulfite, 3 grams p-diethylamine aniline hydrochloride, 25 grams sodium carbonate, and 2 grams potassium bromide, to which about 50 grams urea per liter has been added. After developing with this solution for about 15 minutes, the film is removed and washed for about 10 minutes, and then bleached for about 5 minutes in a 10% solution of potassium ferricyanide. It is then washed for about 5 minutes and placed in a fixing bath of 10% sodium thiosulfate for about 5 minutes, again washed and then dried. The urea accelerates the development of the lowermost layers. The development of the upper layers is also accelerated so that the time of development is reduced.

Referring to Fig. 2, there are illustrated typical curves showing effects of developing a multilayer color film in developer solution containing urea. Curve A shows a typical curve when the development is carried out without the presence of urea, curve B is typical of the effect produced in the first layer, which is the yellow layer and curve C typifies the effect produced in the lowermost or cyan layer. These curves illustrate the marked increase in speed in the cyan layer as compared to the relatively lesser speed increase in the outermost layer. It will be understood that the effect on the intermediate layer in a three layer film will be generally intermediate curves B and C.

I claim:

1. The process which comprises subjecting exposed multilayer silver halide emulsion color film

sensitized to light of the primary colors respectively and containing within the respective layers color formers complementary to the color for which the layer is sensitized to a solution containing amidol and a compound of the following general formula:



wherein X represents a member selected from the group consisting of hydrogen, methyl, allyl and the cyanide radical in a concentration of about 25 to 150 grams per liter.

- 15 2. The process which comprises subjecting exposed multilayer silver halide emulsion color film sensitized to light of the primary colors respectively and containing within the respective layers color formers complementary to the color for which the layer is sensitized to a solution containing amidol and urea in a concentration of about 25 to 150 grams per liter.
- 20 3. The process which comprises subjecting exposed multilayer silver halide emulsion color film sensitized to light of the primary colors respectively and containing within the respective layers color formers complementary to the color for which the layer is sensitized, to a solution containing amidol and about 65 to 75 grams urea per liter.
- 30

HERBERT W. MORREALL, JR.

REFERENCES CITED

35 The following references are of record in the file of this patent:

UNITED STATES PATENTS

| Number       | Name                   | Date          |
|--------------|------------------------|---------------|
| 1,763,990    | Sheppard et al. -----  | June 17, 1930 |
| 2,112,023    | Hosking et al. -----   | Mar. 22, 1938 |
| 2,179,234    | Schneider -----        | Nov. 7, 1939  |
| 2,191,037    | Mannes et al. -----    | Feb. 20, 1940 |
| 2,304,025    | Schneider et al. ----- | Dec. 1, 1942  |
| 2,341,485    | Swan -----             | Feb. 8, 1944  |
| 45 2,363,493 | Baldsiefen -----       | Nov. 28, 1944 |
| 2,404,774    | Dersch et al. -----    | July 30, 1946 |
| 2,410,644    | Fierke et al. -----    | Nov. 5, 1946  |

FOREIGN PATENTS

| Number     | Country             | Date          |
|------------|---------------------|---------------|
| 50 512,060 | Great Britain ----- | Aug. 29, 1939 |